

1

2,702,793

## FOAM-INHIBITING AND FOAM-INHIBITED COMPOSITIONS

William R. Smith, Port Arthur, Tex., assignor to The Texas Company, New York, N. Y., a corporation of Delaware

No Drawing. Application June 13, 1950,  
Serial No. 167,915

1 Claim. (Cl. 252—78)

This invention relates to improvements in foam-inhibiting compositions and foam-inhibited compositions, particularly those compositions containing hydrocarbons.

In certain liquid compositions such as hydrocarbon oils used for the lubrication of engines, in automatic transmissions for automotive vehicles, as hydraulic oils or for similar purposes, the problem of foam or froth has been serious because of the loss of oil due to expansion and overflow, and the starvation of friction surfaces as respects lubrication because of the large proportion of foam content of the oil. Foam or froth has also been a problem in chemical and petroleum processing since large quantities of foam reduce the quantities of material that may be handled in apparatus of predetermined capacity. The various problems involved and some solutions therefore are fully discussed in Patents Nos. 2,416,503 and 2,416,504 issued February 25, 1947, to C. E. Trautman et al., Patent No. 2,375,007 issued May 1, 1945, to R. G. Larsen et al., Patent No. 2,406,671 issued August 27, 1946, to H. Diamond, and Patent Nos. 2,406,971 and 2,407,037 issued September 3, 1946, to F. J. Sowa.

The above patents disclose the use of liquid organo-silicon condensation products or polymers such as silicones or silicates as foam-inhibiting agents in liquids having tendencies to foam, reference being made to the disclosures of such patents for a description of the various compositions used and their methods of preparation and use.

While the compounds disclosed in the foregoing patents have proven generally satisfactory, it is an object of this invention to provide even more efficient foam-inhibiting agents for liquids having foaming tendencies.

Another object of this invention is the provision of a relatively cheap and efficient anti-foaming agent capable of inhibiting foaming of liquids used for special purposes such as in the hydrocarbon oils used in automatic transmissions for automotive vehicles.

Other objects and advantages of the invention will appear from the following description and the accompanying claims.

In brief, the present invention resides in the discovery that an improved foam-inhibiting agent can be formed by the use of liquid organo-silicon condensation products or polymers in combination with a silane. It has been found that by the addition of a small proportion of a silane to the foam-inhibiting agents disclosed in the above patents, a more efficient foam-inhibiting agent can be formed.

The term "silane" as used herein is intended to cover organic derivatives of a hydride of silicon of the type  $\text{SiH}_{2n+2}$ . It is intended to include compounds having the following general formula:



wherein X is R or OR and R represents similar or dissimilar organic radicals such as alkyl, aryl, alkaryl, aralkyl and heterocyclic groups. Typical examples are compounds of the type  $\text{SiR}_4$  such as silicon tetramethyl, silicon tetraethyl, silicon tetraphenyl, silicon tetrabenzyl, and silicon tetrapropyl. Compounds containing mixed radicals, i. e., different aliphatic and aromatic groups are exemplified by tripropylallylsilane. Another type of silane is the alkylsilane such as trimethylsilane, triphenylsilane, triethylsilane, tri-i-butylsilane and tri-i-amylsilane. Other types of silanes are the alkylhalosilanes ranging from trimethylchlorosilane to tribenzylchlorosilane, triethylbro-

2

mosilane to triphenylbromosilane, the fluoroanalogs ranging from triethylfluorosilane to tribenzylfluorosilane, and mixed trialkylchlorosilanes, such as benzylethylpropylchlorosilane.

5 The dialkyldihalosilanes as represented by dimethyl- and diphenyldibromosilane, the alkyltrihalosilanes as represented by methyltrichlorosilane and the alkylalkoxysilanes are also to be included. Examples of the latter class of compounds which is preferred include amyltriethoxysilane, monomethyltriethoxysilane, diisopropyltriethoxysilane, di-n-butyltriethoxysilane, triamylethoxysilane, tri-2-ethylhexylethoxysilane and monolauryltriethoxysilane.

10 The organo-silicon oxide condensation products or condensation products of silanols or organo-silicols referred to herein are intended to include both silicones and silicates, preferably normally liquid, of the following general compositions:



wherein R represents similar or dissimilar organic radicals such as alkyl, aryl, alkaryl, aralkyl and heterocyclic groups; the terminal R's and OR's or other R's and OR's may be substituted by hydroxyl groups; and n is one or more. Such compounds and their methods of preparation to form compounds of different viscosities are well known to the art. Where R in the foregoing formula is an aromatic hydrocarbon grouping, intra-substituents such as a halogen, a nitrogen-containing radical as  $\text{NO}_2$  or  $\text{NH}_2$ , a sulfur-containing radical such as  $\text{SO}_3\text{H}$  or  $\text{SH}$ , or a phosphorus-containing radical such as phosphite, phosphate or the thio derivatives thereof may occur.

15 Typical compounds include dimethyl silicone, methyl phenyl silicone, ethyl butyl silicone, methyl cyclohexyl silicone, dicyclohexyl silicone, diphenyl silicone, hydroxy phenyl methyl silicone, phenyl propyl silicone, phenyl isopropyl silicone, tolyl butyl silicone, tolyl amyl silicone, phenyl hydroxy ethyl silicone and the corresponding polymers of methyl orthosilicate and ethyl orthosilicate. Compounds containing simple organic radicals such as methyl, ethyl and short chain alkyl groups are preferred. Such compounds may have hydroxyl groups or organic radicals 20 as terminals.

25 The compounds are preferably incorporated in the composition to be treated by mixing them with a high boiling naphtha such as kerosine and mixing the resultant combination with the composition.

30 A preferred organo-silicon compound is a dimethyl silicone linear polymer chain-stopped with methyl groups, the silicone being mixed with about 5% very finely divided siliceous material such as finely divided silica. A suspension is formed which is relatively inert in contact with known metals and plastics and is relatively non-inflammable. If desired, the siliceous material may be omitted.

35 The above organo-silicon compounds may range in viscosity from 100 cs. to 250,000 cs., the higher viscosity compounds above 900 cs. being usually preferred.

40 The tests hereinafter described were conducted by the so-called Carnegie Foam Test which has come to be generally recognized as one of the most drastic tests developed thus far. In this test which has been developed primarily for the testing of oils used in hydraulic transmission mechanisms and the like wherein the conditions are ideal for the production of foam, the oil being tested passes through a pump having a submerged intake and an air-open discharge above the body of oil. Simultaneously two propellers are used to agitate the oil body. The oil is heated to a temperature of about 200° F.

45 After the oil is brought to temperature, the propeller motor is turned on and the pump discharge pressure set at 40 lbs. per square inch. After one minute, the motor is shut off and the height of foam, i. e., the distance from the top of the foam to the oil-foam interface, is measured. The foam collapse time is taken as the time elaps-

ing between the stopping of the motor and the first appearances of the oil surface through the foam. The foam height is reported to  $\frac{1}{8}$ " and the foam collapse time to one second. Approximately six quarts of oil is required for the test.

As already described, the present invention is concerned with a foam-inhibitor prepared by mixing a liquid organo-silicon condensation product or polymer with a silane. The results obtained in inhibiting foam by the use of such a combination have proven to be much better than the results obtained by using either type of compound separately. As a matter of fact, silanes per se are of practically no value in inhibiting foam.

As an example of the high and entirely unexpected efficiency of the invention, a hydraulic transmission fluid was prepared with a mineral oil base. About 3.5 to 4.5% of an additive of the methacrylate polymer type, about 2.5 to 3.5% of an additive of the sulfurized sperm oil type and about 0.8 to 1.0% of an additive of a barium thiophosphate-sodium sulfonate type in a light oil as a carrier, all by weight, were added to a base compound formed of a refined paraffin base oil having a viscosity S. S. U. at 100° F. of about 100.

The methacrylate polymer type additive contains approximately 40% of a polymerized ester of methacrylic acid having a molecular weight between 10,000 and 15,000 and of the following general formula:



wherein R is a mixture of cetyl, lauryl and octyl groups. The additive is formed by dissolving the polymer in a Mid-Continent solvent-refined 150 neutral oil. The result is a clear, light-amber colored viscous fluid having a Sp. Gr. 60°/60° F. of 0.89-0.90, and flash point °F., diluted to 10% solids with a S. A. E. 20 oil, COC. of 405 min., a viscosity, Kinematic at 210° F., cs. of 600-800 and a Neut. No. of 0.4 max. This additive has been found valuable as a viscosity index improver and a pour point depressant.

The sulfurized sperm oil type additive can be described as having a sulfurized sperm oil and lanolin base, the principal constituent being a sulfurized derivative of cetyl oleate:



It is probable that the sulfur enters the molecule at the double bond to form a ring structure somewhat as follows:



The additive has a gravity °API of 14.5-16.0; a viscosity S. U. S. at 210° F. of 190 to 230 seconds, and a saponification No. of 140-155. The sulfur content is about 9 to 11% by weight. In addition to functioning as an extreme pressure lubricant, the additive also functions as an oxidation inhibitor and as a mild detergent.

The barium thiophosphate-sodium sulfonate type additive is formed of approximately 12% sodium sulfonate, about 45.5% light lubricating oil as a carrier and about 42.5% of a barium compound of the following type:



wherein  $\text{R}=\text{C}_7+\text{C}_8+\text{C}_{10}$  alcohols. The additive is a dark oily liquid of a density of about 1.016. It contains about 6.0 to 7.3% barium, about 2.6 to 3.2% phosphorus, about 6.0 to 7.0% sulfur, and about 0.25 to 0.40% sodium, all by weight. Its principal function is as an antioxidant.

An anti-foam agent was prepared for the above fluid by adding sufficient kerosine to 10 grams of methyl silicone of 100,000 cs. to make up a total volume of 100 ml. The solution was mixed with the fluid in a proportion to provide a silicone content of 2.5 parts per million.

The fluid was then tested by the Carnegie Foam Test with the following results:

|  | Foam, Inches  | Time, Seconds |
|--|---------------|---------------|
|  | $\frac{1}{8}$ | 41<br>50      |

With another test with only 1.0 p. p. m. silicone, the foam was  $\frac{1}{4}$ " and the time 33 seconds. With the basic oil alone and no anti-foam agent, the foam was  $\frac{1}{2}$ " and the time 35 seconds.

An anti-foam agent according to the teachings of this invention was prepared by adding sufficient kerosine to 10 grams of the same silicone and 20 grams amyltrithoxy-silane a proportion of 1 to 2 by weight to make a total volume of 100 ml. This mixture was added to the same fluid in amounts to make separate samples containing 1.0, 2.5 and 5 p. p. m. silicone (3, 7.5, and 15 p. p. m. of silicone plus silane). These mixtures were tested by the Carnegie Foam Test with the following results.

|    | Silicone (p. p. m.) | Foam, Inches | Time, Seconds |
|----|---------------------|--------------|---------------|
| 30 | 5.0                 | 0            | 0             |
|    | 2.5                 | 0            | 0             |
|    | 1.0                 | 0            | 0             |

From the above, it is evident that silicone without the silane even when used up to 2.5 p. p. m. was only partly effective in inhibiting foam. On the other hand, with as little as 1.0 p. p. m. of the silicone in the silicone-silane combination, there was complete inhibition. On a comparative basis, the silicone-silane combination can be said to be 2.5 times as effective as the silicone alone.

The above-described fluid is a particularly good hydraulic transmission fluid in that it is capable of transmitting power efficiently through either the fluid coupling or torque converter, it is an efficient lubricant for the complicated and precisely machined moving parts such as the various pump units involved, and is capable of satisfactorily lubricating and preventing wear on any gearing contained in the transmission unit. It has the correct viscosity and a pour point of at least -35° F. which satisfies the requirements of temperature extremes liable to be encountered. It is stable in service, resistant to oxidation and deposit formation, and resistant to foam formation and gas entrainment which could interfere with the efficiency of the power transmission.

Application of the invention to other special-purpose oils as well as the usual lubricating oils is also contemplated. One such special-purpose oil is a lubricating oil prepared for use in diesel engines by combining a base oil (having a gravity, API of 22.5-28.5, flash, C. O. C. min. 420° F., fire, C. O. C., min. 470° F., viscosity, S. S. U. at 100° F. of 540-630, viscosity index 76 min., pour point 5° F. max.) with about 16.5% by volume of an additive classified as a basic barium sulfonate, barium dithiophosphate, sulfurized terpene product, the latter being particularly valuable in counteracting the corrosive effects of high sulphur fuels.

Other special-purpose oils include industrial gear lubricants, refrigerator oils and rock-drill lubricants.

It should be noted that the present invention is concerned with the inhibition of gas or air entrainment as well as the inhibition of foam. Foam is the frothy liquid and gas mixture formed on the surface of the liquid. It is readily distinguishable from the liquid proper, the separation taking place at a liquid-foam interface. Air or gas entrainment is not readily determinable and involves an actual increase in the volume of the liquid because of the air or other gas entrained therein. Tests have proven that there may be gas entrainment in the absence of foam.

Use of the foam inhibitor of the present invention is also contemplated in anti-freeze liquids of the type to be added to water in the cooling system of an internal combustion engine or the like such as those liquids prepared from the various types of water-miscible polyhydric alcohols including ethylene and other glycols, poly-

glycols and glycerine. In some instances, the resultant mixtures in the engines have been found to foam to an extent such that the mixture escapes from the cooling system to a degree sufficient to seriously affect the operation of the engine. Consequently, the inhibition of foaming of such mixtures is desirable.

In incorporating such a foam inhibitor in an anti-freeze mixture, such as one of the ethylene glycol type, reference being made to the co-pending applications of T. C. Heisig, Serial No. 84,259, filed March 29, 1949, now abandoned, and Serial No. 138,513, filed January 13, 1950, for a more complete description thereof, the glycol if such used, is usually mixed first with any desired corrosion inhibitors in water solution to provide a mixture containing about 92 to 97% glycol. The organic-silicon compound and the silane may then be blended with a suitable hydrocarbon to obtain the final specific gravity desired, and the resultant anti-foam mix added to the glycol and water mixture in an amount between 0.90 and 1.25%, preferably about 1.05% by volume. The resultant anti-freeze is subsequently mixed with from 1 and 1/2 to 4 times its volume of water to provide the final coolant dependent upon the desired depressing of the freezing point of the coolant.

In addition to the above, the anti-foam agents herein described may be used in other types of hydrocarbon compositions including special solvents, gasoline, kerosine, cleaning fluids and turbine oils. Their use is also contemplated in such substances as latex, resins, paints, perfumes, synthetic and natural oils, vegetable oils and fats, animal oils and fats and cutting oils such as those of the soluble type which contain emulsifying agents and are diluted with water.

Their use is also contemplated in connection with foaming as found in oil and the water emulsions, in connection with the various processing steps of various substances such as distillation, fraction, concentration, filtration, solvent extraction, emulsion breaking, evaporation and condensation.

In summarizing, it is believed evident from the above that applicant has provided a new and exceedingly effi-

cient foam inhibitor. In addition it should be noted that the silane in the inhibitor is a much cheaper ingredient than the organo-silicon compounds, this making the final composition cheaper than those used heretofore.

5 The reasons for the high and unexpected efficiency of the combinations of the invention are not understood. It may be that there is some chemical reaction between the silane and the organo-silicon compound productive of an entirely new compound. Therefore the terms mixture, 10 composition or combination as used herein and in the claim is intended to cover both physical and chemical combinations of the various compounds used.

Obviously many modifications and variations of the invention, as hereinbefore set forth, may be made without departing from the spirit and scope thereof and, therefore, only such limitations should be imposed as are indicated in the appended claim.

I claim:

20 A composition of matter of reduced foaming and gas entraining properties consisting essentially of a mineral oil characterized by a tendency to foam and entrain gas when agitated, and 3 to 15 p. p. m. of a foam and gas entraining inhibitor consisting essentially of both 100,000 25 cs. dimethyl silicone and amyl triethoxysilane, said silicone and said silane being present in a proportion of 1:2 by weight.

#### References Cited in the file of this patent

#### UNITED STATES PATENTS

|    |           |                       |               |
|----|-----------|-----------------------|---------------|
| 30 | 2,129,281 | Lincoln et al. -----  | Sept. 6, 1938 |
|    | 2,375,007 | Larsen et al. -----   | May 1, 1945   |
|    | 2,406,671 | Diamond -----         | Aug. 27, 1946 |
| 35 | 2,416,503 | Trautman et al. ----- | Feb. 25, 1947 |
|    | 2,416,504 | Trautman et al. ----- | Feb. 25, 1947 |
|    | 2,435,124 | Bollinger -----       | Jan. 27, 1948 |
|    | 2,462,999 | Scott -----           | Mar. 1, 1949  |
|    | 2,468,869 | Daudt -----           | May 3, 1949   |
|    | 2,490,068 | Lincoln et al. -----  | Dec. 9, 1949  |
| 40 | 2,491,833 | Sauer -----           | Dec. 20, 1949 |
|    | 2,561,178 | Burkhard -----        | July 17, 1951 |